

3,177,143  
EMULSION FOR THE CONDITIONING OF  
RAW COTTON FIBERS

Frederick T. Lense, Mauldin, S.C., assignor to Esso Research and Engineering Company, a corporation of Delaware  
No Drawing. Filed Aug. 29, 1961, Ser. No. 134,568  
5 Claims. (Cl. 252—8.9)

This invention relates to the use of branched chain alcohols and emulsions thereof in fiber processing. The invention is applicable to the conditioning of raw cotton, organic derivatives of cellulose, and other fibers having wettability characteristics equivalent to such fibers, but is especially directed to the conditioning of lint cotton fibers prior to spinning.

This is a continuation-in-part of application Serial Number 815,327, filed May 25, 1959 and application Serial Number 815,322, also filed on May 25, 1959, both now abandoned.

In the processing of such raw textile fiber stock, it has heretofore been customary to apply, as by spray or wiping action, a conditioning fluid, such as a mineral oil or an oil compounded with modifying substances, to the raw fibers, after they have been separated from the raw mat, to facilitate the subsequent operations of forming them into yarn or thread. For example, in the processing of cotton, the bale of raw cotton is usually passed to a bale breaker and cleaner, where the raw mat is formed and dirt and dust are largely removed. The resulting mat is then passed to a picker where a beater roll separates the raw cotton fibers from the mat. The separated fibers are then subjected in series to the usual carding, drawing and roving operations, and finally to spinning to form yarn or thread. The latter then passes to the looms where the weaving operation is carried out to form cloth.

The conditioning treatment of the raw fibers by the conditioner fluid application may take place when the bale is opened or at any subsequent step leading to the spinning operation per se as, for instance, at the beater roll of the picker immediately after the fibers have been separated from the mat.

The term "spinning" in the broad sense refers collectively to all of the operations in manufacturing a yarn from fibrous raw material. The specific operation known as spinning may be defined as the operation of drafting roving to the required counts, inserting the required number of turns per unit of length in the yarn, and winding it into the form of a cop or onto a bobbin or spool. Since the specific discussions herein relate to the processing of natural fibers the term "spinning" is used herein in accordance with the later, more narrow definition. It is to be understood that in the processing of synthetic fiber the term is used to include the extrusion of a spinning solution through spinnerettes to form filaments.

It is the object of such treatment to reduce fly and dust in the carding room, to increase the flexibility and pliability of the fibers for the subsequent operations with a view to producing a higher percentage of long fibers and fewer short or broken fibers, and to reduce the generation of static electricity in the subsequent processing without requiring excessive humidification.

The conditioners having a mineral oil base have not been entirely satisfactory. It has been found that their use in many instances results in an objectionable degradation in tensile strength of the spun yarn. These conditioners have also presented problems of fiber discoloration.

Likewise, the straight chain higher aliphatic alcohols, such as stearyl and oleyl alcohols, leave a solid residue that is objectionable because it is difficult to remove from

the fibers and therefore adversely affects their dyeing characteristics.

It has now been found that a new source of fiber conditioners can be prepared from certain high molecular weight alcohols.

Therefore, this invention relates in particular to the use of branched chain,  $C_{13}$  to  $C_{32}$ , particularly  $C_{16}$  to  $C_{26}$ , and preferably  $C_{16}$  to  $C_{20}$ , monohydric alcohols which are liquid at room or field temperatures above about 40° F., as lubricants and anti-static agents in the carding, drawing, spinning, twisting, coning, pirning, hanking, weaving, knitting and associated mechanical operations of fiber processing.

One aspect of the invention relates to the use of these alcohols in fiber processing. Another aspect of the invention relates to the use of 25 to 75 wt. percent aqueous emulsions of these alcohols containing an emulsifying agent which does not impart substantial wettability to the emulsion in the carding, drawing, and spinning of cotton fibers.

The preferred emulsion for use in the aforesaid processes are relatively stable aqueous emulsions of the afore-described alcohols which may be formed by simple agitation with low concentrations of an emulsifier compound having an organic hydrophobic component and a poly-alkylene oxide hydrophilic component wherein the weight relationship between such components is balanced in a manner that will not impart substantial wetting properties to the emulsifier.

It is known that higher molecular weight alcohols are not emulsifiable in or with water unless an emulsifying agent is added.

Providing the wetting properties of the emulsifier are sufficiently low, concentrations of emulsifier may be used in accordance with this invention up to as high as 10 wt. percent based on the weight of water in the emulsion. Obviously, however, much lower concentrations, e.g. 0.05 to 1.0, preferably below 0.2 wt. percent, are preferred, both with regard to cost and with regard to the aforementioned wetting properties. The preferred emulsions may be effected by simple agitation and remain stable for periods adaptable for diversified use, e.g. from 1 to 24 hours, and be reformed after de-emulsification in the same manner. Emulsions of the aforescribed ingredients which will remain stable for much longer periods can be effected by homogenization, colloid milling and ultrasonic devices known to the art.

The alcohols or emulsions may be applied to cotton fibers in amounts up to about 10 wt. percent of the said fibers without wetting such fibers to a degree that will deleteriously affect the subsequent use of such fibers in conventional, mechanical textile processing operations. For most purposes it will be found that about 0.2 to 10 wt. percent of the liquid is satisfactory. Even very small amounts, e.g. 0.05 wt. percent of the fiber, have a noticeable effect. However, applications from about 0.5 to 2.0 wt. percent are preferred.

Suitable alcohols for use in this invention are preferably prepared by the Aldox process, a modification of the well-known Oxo process.

In the Aldox process, a primary alcohol product is prepared from an olefin and a synthesis gas of carbon monoxide and hydrogen. Except for the use of a reaction modifier hereinafter discussed, and the product, the Aldox process is substantially the same as the Oxo process. In the Oxo process, oxygenated organic compounds are synthesized in the presence of a cobalt catalyst from organic compounds containing olefinic linkages by reaction with carbon monoxide and hydrogen. In this reaction, predominantly aldehydes and minor proportions of ketones and alcohols are formed. The products from this Oxo step may then be hydrogenated in a second step to con-

vert the organic carbonyl compounds containing one more carbon atom than the olefinic starting material to the corresponding alcohol. The hydrogenation catalyst may comprise any known reduction catalyst such as metallic supported or unsupported nickel, copper chromite, sulfactive catalyst such as oxides and sulfides of tungsten, nickel, molybdenum and the like.

Straight and branched chain olefins such as propylene, butylene, pentene, hexene, heptene, styrene, olefin polymers such as di and triisobutylene, hexene and heptene 10 dimers, polypropylenes, olefinic fractions from the hydrocarbon synthesis process, thermal or catalytic cracking operations, and other sources of hydrocarbon fractions containing such olefins may be used as starting materials 15 depending on the nature of the final product desired. The synthesis gas mixture fed to the first stage may be any desired ratio of  $H_2$  to  $CO$ , preferably within the limit of 0.5 to 2 volumes hydrogen per volume of carbon monoxide. The conditions for reacting olefins with the synthesis gases vary somewhat in accordance with the nature 20 of the olefin feed, the reaction being generally conducted at pressures in the range of from about 1500 to 4500 p.s.i.g. and the ratio of synthesis gas to olefin may vary widely; in general about 2500 to 25,000 cubic feet of  $H_2+CO$  per barrel of olefin feed are employed.

The catalyst for the first stage of the process may be employed in the form of an oil-soluble compound of the catalytically active carbonylation metal. Thus, there have been employed the salts of the metals such as cobalt and a high molecular weight fatty acid such as stearic, oleic, 30 naphthenic, linoleic and the like. Water-soluble catalyst, such as cobalt acetate, chloride, and the like, may also be used. Catalyst concentrations may vary from about 0.05 to 1.0% by weight of the catalyst calculated as cobalt on olefinic feed. The first stage for carbonylation reaction 35 may be carried out at temperatures in the range of from about 250° to 450° F. depending upon the nature of the olefin and other reaction conditions. In general, the lower olefins will react at lower temperatures and will react to a greater extent than the higher molecular weight olefins. 40

The Oxo process without modification will produce some alcohols of higher molecular weight, but the yields of such products are relatively low. These alcohols result from several different mechanisms including aldolization, dehydration, dimerization, acetalization, etc. Some of these alcohols contain two more than twice the number of carbons in the olefin feed and are highly branched alkanols. Another type contains three more than twice the number of carbons in the olefin feed but this latter type also contains an additional oxygen atom in the molecule forming an ether linkage with two internal carbon atoms.

For a more detailed description of these ether alcohols see "Oxo Ether Alcohols," Bartlett et al., "Industrial and Engineering Chemistry," March 1959, pages 257-258.

In the Aldox process the same reactors, catalyst, and reaction conditions may be employed as in the aforesaid Oxo process, and, in addition, a reaction modifier is employed which results in the production, in high yields, of a primary alcohol product having  $2n+2$  carbon atoms, where an olefin with  $n$  carbon atoms is passed to the carbonylation zone. Accompanying this reaction is the normal aldehyde reaction producing aldehydes and alcohols having  $n+1$  carbon atoms.

The aforesaid reaction modifiers are preferably zinc compounds. The zinc compounds suitable are salts or fatty acids, oxides, hydroxides, carbonates, and also metallic salts of cobalt hydrocarbonyl. Thus, in the Aldox process there is passed into the first-stage reaction zone 70 along with the olefin carbon monoxide, hydrogen, and cobalt carbonylation catalyst, a reaction modifier, preferably zinc. Other Aldox modifiers have been suggested in the prior art.

The mono-ether, mono-hydroxy alcohols hereinbefore 75

described may also be produced in the Aldox process in somewhat lesser quantities. The  $C_{13}$  to  $C_{32}$  alcohols of this group may also be used in this invention.

A liquid oxygenated reaction product comprising aldehydes from the carbonylation reaction containing inorganic contaminants, e.g. dissolved cobalt carbonyl and zinc salts, is sent to a catalyst decomposition or decobalt-ing zone, where in the presence of heat and steam, water, or dilute organic acid, the inorganic contaminants are removed from the aldehyde product in a manner known in the art. This product, now substantially completely free of inorganic compounds, is hydrogenated under conventional conditions to alcohols and the alcohol product fractionated to produce both the  $n+1$  and  $2n+2$  alcohols, as described.

The production of such alcohols by the Aldox process is covered by U.S. Patent 2,811,567.

Monohydric, primary alcohols may also be prepared from aldehydes via conventional Aldol condensation. By this process the positive end of a carbonyl group is linked with a carbanion by a typical "aldol condensation" known to the art. The primary Aldol product may then be dehydrated by means known to the art to yield an unsaturated aldehyde which can be hydrogenated to a primary alcohol.

Another method for preparing monohydric, primary alcohols is by the process known to the art as the Guerbet reaction.

Particularly suitable emulsifiers for use with this invention are those having a hydrocarbon comprising hydrophobic group containing 20-60, preferably 20-36, carbon atoms and a polyalkylene oxide hydrophilic group which constitutes from 50-95, preferably 70-95 wt. percent of the emulsifier. In the emulsifiers of this type, the hydrocarbon comprising group may be an alkyl, aryl, or alkylaryl hydrocarbon or a substituted alkyl, aryl or alkylaryl hydrocarbon, e.g. ethers and alcohols. Many emulsifiers of this type are sold commercially and may be prepared by various methods well known to the art. A particularly good emulsifier for this purpose is marketed under the trade name of Igepal DM-880. The alkylene oxide units in the hydrophilic group may be either ethylene oxide or propylene oxide with the former preferred. Of these, the most preferred are dialkyl phenoxy polyoxyethylene ethanol type non-ionic emulsifiers wherein the alkyl substituents of the phenol nucleus contain at least 9 carbon atoms each and the ethylene oxide units comprise 75-95 wt. percent of the compound. With the most preferred type of emulsifier just described, the emulsions of this invention may be effected with emulsifier concentrations in the range of 0.05 to 0.2%, preferably 0.075 to 0.125%, based on the weight of water in the emulsion. Such emulsifiers have the added advantage that they may be used with the alcohols of this invention in much larger quantities, i.e. above 1%, if desired, without producing a noticeable increase in the wetting properties.

Another variation of this type of emulsifier which does not impart substantial wettability to the alcohols of this invention may also be prepared wherein the hydrophobic element is a polyoxyalkylene, e.g. polyoxypropylene, polymer prepared by the condensation of propylene oxide, or a higher alkylene oxide, e.g. butylene oxide, with an organic base compound containing at least one and preferably a plurality of reactive hydrogen atoms, e.g. propylene glycol, monofunctional alcohols such as butanol, secondary amines such as diethyl amine, etc., and the hydrophilic group is formed by condensing ethylene oxide with the aforesaid hydrophobic element.

Emulsifiers of this general type are discussed in detail in U.S. Patents 2,674,619 and 2,677,700, and elsewhere in the literature. See "Soap and Sanitary Chemicals" (1950), vol. 26, No. 10, beginning at page 40; "The Journal of the American Oil Chemists Society" (1951), vol. 28, beginning at page 294; and vol. 29 (1952), of

the same publication beginning at page 240. These emulsifiers may be tailored to specific uses by controlling the hydrophobic-hydrophilic balance and the molecular weight of both the hydrophobic and hydrophilic groups.

Thus, the advantages to be gained by emulsifying water and higher molecular weight alcohols such as hereinbefore described with the emulsifiers described herein are at least twofold. First, an emulsifier is employed which adds little or nothing to the wetting properties of the alcohol and water per se and, second, stable emulsions can be effected with extremely low concentrations of the emulsifier thereby minimizing any potential increase in wetting properties. Neither water nor higher molecular weight alcohols such as those hereinbefore described will "wet out" cotton fibers under ordinary conditions of temperature and pressure when applied in the range of 0 to 10 wt. percent based on the weight of cotton fibers.

A convenient reference which may be used to characterize an emulsifier that will "impart substantial wettability" to the emulsions is provided by identifying the undesirable emulsifier as one that will reduce the wetting time of a  $C_{20}$  branched chain, monohydric, primary alcohol-water emulsion below about 15 minutes as measured by Standard Test Method 17-1952 set forth in the 1958 Technical Manual of the American Association of Textile Chemists and Colorists at page 152 using standard test skeins of 2-ply cotton yarn, 0.1 wt. percent emulsifier based on weight of water, and a 25/75 water to alcohol weight ratio.

The term "branched chain, monohydric, primary alcohol" as used herein shall be construed to include both monohydric, primary alcohols which aside from the hydroxyl group are composed exclusively of carbon and hydrogen atoms and monohydric, primary alcohols which aside from the hydroxyl group are composed of carbon atoms, hydrogen atoms and a single oxygen atom forming an ether linkage with two of such carbon atoms.

#### Example I

A branch chain  $C_{16}$  monohydric alcohol wherein the carbinol group is positioned intermediate to the ends of the longest carbon chain was prepared by the Aldox process. This process and the range of operating conditions within which it may be carried out had previously been discussed herein. The alcohol of this example was prepared by this process employing as the olefin feed a  $C_7$  olefin fraction previously prepared by a U.O.P. type polymerization of a  $C_3$  to  $C_4$  olefin stream, cobalt and zinc catalyst in the form of their oil-soluble fatty acid salts, i.e. oleates, and under the following operating conditions.

##### Carbonylation reaction:

$C_7$  olefin feed rate \_\_\_\_ 510-530 b./d.  
 Catalyst concentration \_\_\_\_ .08 wt. percent cobalt (on olefin), .02 wt. percent zinc (on olefin).  
 Temperature, ° F. \_\_\_\_ 350-360.  
 Pressure, p.s.i.g. \_\_\_\_ 3000-3500.  
 Ratio of  $H_2$  to CO in synthesis gas mixture \_\_\_\_ 1:1.4:1.  
<sup>1</sup> Barrels per day.

The aldehyde comprising reaction product was subjected to a conventional decobalting treatment to remove inorganic contaminants. The decobalting was carried out at temperatures averaging about 270-380° F., pressures averaging about 155 to 165 p.s.i.g., in the presence of water employed in a water to feed ratio of about 0.1 to 1.

The aldehyde comprising product now substantially completely free of inorganic compounds was hydrogenated by conventional methods to alcohols, i.e. at an average temperature of about 470° F. and a pressure of about 3000 to 3500 p.s.i.g., and subsequently fractionated to separate the aforesaid  $C_{16}$  alcohol.

A 25/75 wt. percent of water/alcohol was prepared by blending the  $C_{16}$  alcohol prepared above with water and 0.1 wt. percent based on said water, of a commercially available non-ionic emulsifying agent comprising a dinonyl phenol alkylene oxide condensate containing about 85 to 90 wt. percent ethylene oxide per molecule.

In a textile spinning mill where raw bale cotton is blended, sprayed with a fiber lubricant, matted, carded into rovings, and then spun into yarn and threads, tests were conducted with the above-described alcohol emulsions. Other tests were conducted using a commercially available fiber lubricant having a hydrocarbon base. The latter lubricant was being used for this purpose by the mill at the time the tests were conducted.

In each test the lubricant was placed in a storage tank from which it was fed by separate proportioning pumps into spray nozzles attached to fine cotton openers. Each opener handles about 125 lbs./hr. of raw baled cotton. About 0.5 to 0.75 wt. percent of lubricant was added in each test. The lubricated cotton was then blended, mat rolled, transferred to the carding machines and subsequently spun into yarn. A major proportion of the trash included with the lint cotton is removed at the carding step.

With regard to the cotton sprayed with the aforesaid alcohol emulsion, the following observations were made.

(1) No problems resulting from a build-up of static electricity were detected.

(2) The appearance of the alcohol sprayed cotton with relation to cleanliness was improved, indicating more trash removal.

(3) The alcohol sprayed cotton demonstrated a luster not evident with that sprayed with hydrocarbon comprising lubricant.

(4) The alcohol sprayed cotton demonstrated a better evenness in the yarn and fewer slubs in the card web. The average reduction in these when compared to the cotton sprayed with the hydrocarbon comprising lubricant was in the order from 9 to 6, an improvement of roughly 50%.

The term "sub" as used herein refers to a soft, thick uneven place in a yarn.

#### Example II

Cotton is sprayed with an emulsion prepared as in Example I from a  $C_{20}$  branched chain, monohydric, primary alcohol made in accordance with the method described in the aforementioned example while using a  $C_9$  olefin feed. The cotton is blended, mat rolled, carded and subsequently spun into yarn and thread. The results are comparable to those obtained in Example I.

#### Example III

Cotton is sprayed, as described in Example I, with a  $C_{16}$  branched chain, monohydric, primary alcohol prepared in accordance with Example I. The cotton is blended, mat rolled, carded and subsequently spun into yarn and thread. The results are comparable to those obtained with the emulsion in the aforementioned example.

#### Example IV

Cotton is sprayed, as described in Example I, with a  $C_{20}$  branched chain, monohydric, primary alcohol prepared in accordance with Example I. The cotton is blended, mat rolled, carded and subsequently spun into yarn and thread. The results are comparable to those obtained with the emulsion in the aforementioned example.

What is claimed is:

1. An emulsion consisting essentially of 25 to 75 wt. percent of a  $C_{16}$  to  $C_{20}$  branched chain, monohydric, primary alcohol containing 25 to 75 wt. percent water and 0.05 to 10 wt. percent, based on said water, of a non-ionic emulsifying agent containing a hydrophobic group consisting of a dialkyl substituted phenol containing 20 to 36 carbon atoms wherein each alkyl substituent contains at least 9 carbon atoms and a polyalkylene oxide

hydrophilic group comprising 70 to 95 wt. percent of said agent, wherein said alcohol is a liquid at temperatures between 40° and 115° F.

2. An emulsion in accordance with claim 1 wherein said polyalkylene oxide is a polyethylene oxide condensate. 5

3. An emulsion in accordance with claim 1 wherein said polyalkylene oxide comprises between 85 and 95 wt. percent of said agent.

4. An emulsion in accordance with claim 1 wherein said emulsion contains 0.075 to 0.125 wt. percent of said 10 emulsifying agent based on the weight of said water.

5. An emulsion in accordance with claim 1 wherein

said emulsifying agent is a dinonyl phenol ethylene oxide condensate.

References Cited by the Examiner

UNITED STATES PATENTS

|           |       |                |            |
|-----------|-------|----------------|------------|
| 2,054,257 | 9/36  | Hueter         | 252—312 XR |
| 2,132,348 | 10/38 | Bertsch        |            |
| 2,150,568 | 3/39  | Whitehead      |            |
| 2,677,700 | 5/54  | Jackson et al. | 260—488    |

WILLIAM D. MARTIN, *Primary Examiner.*

RICHARD D. NEVIUS, *Examiner.*